# EUROPEAN PATENT SPECIFICATION

(11) **EP 1 164 413 B1**
(45) Date of publication and mention of the grant of the patent: **02.11.2006**
(21) Application number: 01201989.9
(22) Date of filing: 28.05.2001
(51) Int. Cl.: G03C 1/06

(54) **High contrast photographic element containing a nucleator**
Einen Keimbildner enthaltendes kontrastreiches photographisches Element
Elément photographique à haut contraste contenant un agent de nucléation

(30) Priority: 12.06.2000 GB 0014329
(43) Date of publication of application: 19.12.2001
(73) Proprietor: EASTMAN KODAK COMPANY, Rochester, New York 14650 (US)
(72) Inventor: Bogie, Judith Anne, Middlesex HA1 4TY (GB); Coldrick, Philip John, Middlesex HA1 4TY (GB); Goddard, John DeMita, Middlesex HA1 4TY (GB); Leyshon, Llewellyn James, Middlesex HA1 4TY (GB)
(74) Representative: Haile, Helen Cynthia

(56) References cited:
- US-A- 5 858 610
- PATENT ABSTRACTS OF JAPAN vol. 017, no. 631 (P-1648), 22 November 1993 (1993-11-22) & JP 05 204076 A (KONICA CORP), 13 August 1993 (1993-08-13)
- DATABASE WPI Section Ch, Week 199427 Derwent Publications Ltd., London, GB; Class E19, AN 1994-223114 XP002178899 & JP 06 161009 A (DAINIPPON INK & CHEM KK) , 7 June 1994 (1994-06-07)

## Description

### FIELD OF THE INVENTION

This invention relates to high contrast photographic silver halide materials and in particular to those of the graphic arts type and is related to copending European Patent application no. 99204096.4 published as EP1008902.

### BACKGROUND OF THE INVENTION

In the field of graphic arts, an ultrahigh contrast photographic material is required for achieving satisfactory halftone dot reproduction of a continuous tone or reproduction of a line image in the process of making a lithographic printing plate. For many years these ultrahigh contrast photographic images were obtained by developing a 'lith' emulsion (usually high in silver chloride content) in a hydroquinone, low sulphite, 'lith' developer by the process known as infectious development. However, such low sulphite developers are inherently unstable and are particularly inappropriate for machine processing.

More recently an image formation system providing ultrahigh contrast where the gamma (contrast) exceeds 10 has been provided conventionally in a material wherein silver halide bearing a surface latent image is developed in the presence of a hydrazine (also known as a nucleating agent), specifically an acylhydrazine, which can be incorporated into the photographic material or into the developer. The pH of the developer solution is usually in the range 10.0 to 12.3, typically about 11.5, and the developer includes conventional amounts of sulphite, hydroquinone and possibly metol or a pyrazolidone. While such a process is better than the low sulphite lith' process, the developer still has a high pH requirement for it to function correctly. Such a solution is not as stable as is desirable. Additionally, high pH solutions are environmentally undesirable because of the care needed in handling and disposing of the effluent.

Unfortunately, light sensitive materials whose contrast is enhanced by the presence of a hydrazine nucleating agent show large variations in their photographic properties as the developer is exhausted or through the course of time, for example as the pH of the developer varies and in particular as the pH is lowered. The pH of the developer can vary for a number of reasons: for example, exhaustion and absorption of carbon dioxide causes the pH to drop whilst air oxidation causes the pH to rise, as can concentration through evaporation.

It is also known that a developer solution having a pH below 11 can be employed by using certain hydrazides active at this pH. Hydrazides proposed for such use are described, for example, in US Patent Nos. 4,278,748; 4,031,127; 4,030,925 and 4,323,643 and in EP-A-0 333 435. A nucleator containing both a hydrazide moiety and a nicotinamide moiety is disclosed in US Patent No. 5,288,590.

Developer solutions with these low pHs can also be used by the introduction of a contrast-promoting agent (commonly called a booster) to give adequate activity. The booster can be incorporated into the photographic layer or may be dissolved in the developer solution. The booster may be, for example, one of the boosters as described in US Patent No. 5,316,889 or an amine booster as described in US Patent Nos. 4,269,929; 4,668,605, 4,740,452 or EP-A-0 364 166. Compounds bearing different functionalities e.g. phosphonium and pyridinium, have also been shown to be active, as described in US Patent No. 5,744,279.

The disadvantages connected with the necessity of using a booster to promote nucleation are numerous. Some materials are toxic, some are excessively volatile, some have unpleasant odours, some tend to form azeotropes with water, some build up in the developer during processing, some are insufficiently soluble in an aqueous alkaline photographic developing solution and some are costly, yet must be used at a relatively high concentration, thereby contributing substantially to the overall cost of the material. Moreover, many boosters exhibit a degree of activity as contrast-promoters that is less than is desired for commercial operation. In addition, a photographic system depending on the combination of nucleator and booster is an exceedingly complex system which makes its performance particularly sensitive to variation. It would be desirable therefore if good nucleation could be achieved in the absence of such a booster or with a reduced amount of such a booster.

In the non-image areas on the processed film unwanted small dots can appear and this is called 'pepper fog'. This is due to unintentionally fogged grains developing and being amplified by the nucleation process and being rendered visible. Nucleators which are unstable or more active and diffuse more rapidly can result in more and larger pepper fog spots. In high contrast materials therefore a balance needs to be achieved between vigorous development and pepper fog.

Another consideration is chemical spread (or image spread) which is a measure of the increase in size of developed dots or lines produced by nucleation of the edge of the image area causing development of the image boundary beyond the original exposed edge. This spread is small but measurable and can reduce the resolution of very fine lines.

### PROBLEM TO BE SOLVED BY THE INVENTION

The problem is therefore to provide a nucleator for incorporation into a photographic material or into the developer which gives ultrahigh contrast but which at the same time shows less sensitivity to variations in the developing conditions, such as pH or development time, provides sufficient activity in the presence of reduced amounts of a booster or ideally in the absence of booster, provides lower chemical spread and has significantly reduced pepper fog in the photographic material.

It has been found that these objectives can be achieved by the use of a nucleating agent comprising (a) two nicotinamide moieties, which may be the same or different, which are linked by a linking group, and (b) a hydrazide moiety linked to only one of those nicotinamide moieties. Such a nucleating agent can lead to unexpectedly good nucleation even in the absence of a booster and also in a developer whose pH is variable, with concomitant lower chemical spread and pepper fog.

### SUMMARY OF THE INVENTION

According to the present invention therefore there is provided an ultrahigh contrast photographic material comprising a support bearing a silver halide emulsion layer, containing a hydrazide nucleating agent in the emulsion layer or a hydrophilic colloid layer, characterised in that the nucleating agent of formula (I) has one of the following formulae:-
wherein Z¹ and Z² are the same or different and each is a nicotinamide residue, at least one of which is positively charged;
Y is a substituted aryl or heterocyclic ring;
one of A₁ and A₂ is a hydrogen atom and the other is a hydrogen atom, an acyl group or an alkyl- or aryl-sulfonyl group, any of which groups may be substituted;
BG is a blocking group;
L is a linking group;
T is an anionic counterion
and n is 1 or 2.

In another aspect of the invention there is provided an ultrahigh contrast photographic material comprising a support bearing a silver halide emulsion layer, containing a hydrazide nucleating agent in the emulsion layer or a hydrophilic colloid layer, characterised in that the nucleating agent of formula (I), as hereinbefore defined, is in combination with a nucleating agent of formula (II), which comprises a dimeric molecule comprising two monomers linked by a linking group, each monomer of which (a) may be the same or different and (b) comprises a hydrazide moiety and a nicotinamide moiety.

In a further aspect of the invention there is provided an ultrahigh contrast photographic material, as hereinbefore defined, which also contains in the emulsion layer or a hydrophilic colloid layer, a booster compound, as hereinafter defined.

In yet another aspect of the invention there is provided a process of forming a photographic image having ultrahigh contrast which comprises imagewise exposing a photographic material comprising a support bearing a silver halide emulsion layer and processing it with an alkaline developer solution, characterised in that it is developed in the presence of a nucleating agent comprising either a compound of formula (I), as hereinbefore defined, or a compound of formula (I) in combination with a compound of formula (II), as hereinbefore defined, optionally in the presence of a booster compound, as hereinafter defined.

### ADVANTAGEOUS EFFECT OF THE INVENTION

The nucleating agents for use in the invention show less sensitivity to variation in the development conditions than do conventional nucleating agents, leading to significant improvements in processing robustness. Furthermore they are found to provide sufficient activity in the presence of less than the normal amount of booster or even in the absence of such a booster, with cost and environmental advantages. Additionally they provide lower chemical spread and significantly reduced or no observable pepper fog in the photographic material.

A further benefit resides in that, when the synthesis provides both a compound of formula (I) and a compound of formula (II), the products thereby obtained can be used directly, without the necessity of a separation step, leading to a cost advantage.

### DETAILED DESCRIPTION OF THE INVENTION

The nucleators of formula (I) for use in photographic materials of the invention have one of the following general formulae:-
wherein Z¹ and Z² are the same or different and each is a nicotinamide residue, at least one of which is positively charged;
Y is a substituted aryl or heterocyclic ring;
one of A₁ and A₂ is a hydrogen atom and the other is a hydrogen atom, an acyl group or an alkyl- or aryl-sulfonyl group, any of which groups may be substituted;
BG is a blocking group;
L is a linking group;
T is an anionic counterion
and n is 1 or 2.

The nucleators of formula (II), which may be used in combination with a nucleator of formula (I), preferably have one of the following general formulae:- or
wherein each monomer linked by linking group L is the same or different;
Z is a positively charged nicotinamide residue; and
Y, A₁, A₂, BG, L and T are as defined for a compound of formula (I).

In a preferred embodiment each of A₁ and A₂ in compounds of formula (I) and (II) is a hydrogen atom.

More preferably the nucleating agent of formula (I) has one of the following formulae A, B or C, formula A being the most preferred:-

More preferably the nucleating agent of formula (II) has one of the following formulae D, E or F, formula D being the most preferred.

In these embodiments,
eachR₁CO comprises a blocking group and in particular each R₁, which in the compound of formula (II) is the same or different, is independently selected from a hydrogen atom, and an unsubstituted or substituted alkyl, aryl, alkoxy, aryloxy, alkoxy- or aryloxy-carbonyl and alkyl- or aryl-aminocarbonyl group; or each R₁ is or contains an unsubstituted or substituted heterocyclic group, having a 5- or 6-membered ring containing at least one nitrogen, oxygen or sulfur atom, wherein the ring may be linked either directly to the carbonyl group or via an alkyl, alkoxy, carbonyl, amino- or alkylamino-carbonyl group and wherein the ring may be fused to an unsubstituted or substituted benzene ring;
each R₂ and R₃, which in a compound of formula (II) are the same or different, is independently selected from hydrogen and an unsubstituted or substituted alkyl or aryl group and p is 0 or 1;
each R₄ and R₅, which in a compound of formula (II) are the same or different, and each R₆, which may be the same or different, is independently selected from hydrogen, halogen, hydroxy, cyano and an unsubstituted or substituted alkyl, aryl, heterocyclyl, alkoxy, acyloxy, aryloxy, carbonamido, sulfonamido, ureido, thioureido, semicarbazido, thiosemicarbazido, urethane, quaternary ammonium, alkyl- or aryl-thio, alkyl- or aryl-sulfonyl, alkyl- or aryl-sulfinyl, carboxyl, alkoxy- or aryloxy-carbonyl, carbamoyl, sulfamoyl, phosphonamido, diacylamino, imido or acylurea group, a group containing a selenium or a tellurium atom and a group having a tertiary sulfonium structure;
each m is the same or different and is an integer from 0 to 4;
each q, which in the compound of formula (II) is the same or different, is an integer from 0 to 4;
each R₇ is the same or different and is independently selected from hydrogen and an unsubstituted or substituted alkyl or aryl group;
each X, which in the compound of formula (II) is the same or different, is independently selected from C, S=O and C-NH;
each (link₁), which in the compound of formula (II) is the same or different, is independently selected from an unsubstituted or substituted alkylene, polyalkylene, aryl, arylaminocarbonyl or heterocyclyl group and each n is 0 or 1; and
each (link₂) is a linking group independently selected from an unsubstituted or substituted polyalkylene, polyalkylene oxide, polyalkylene containing one or more heteroatoms selected from nitrogen, oxygen and sulfur, separated from each other by alkylene groups, or an unsubstituted or substituted polyalkylene in which the alkylene groups are separated by an unsubstituted or substituted aryl or heterocyclic ring and
T⁻ is an anionic counterion.

As used herein and throughout the specification the term alkyl refers to an unsaturated or saturated straight or branched chain alkyl group (including alkenyl) having 1-20 atoms and includes cycloalkyl having 3-8 carbon atoms. The term aryl includes aralkyl (and specifically fused aryl within its scope). The term heterocyclic specifically includes fused heterocyclic within its scope. The term polyalkylene is defined as the group (CH₂)ₙ wherein n is an integer from 2 to 50.

The term 'blocking group' refers to a group suitable for protecting the (hydrazine) group but which is readily removable when necessary.

It is preferred that R₁ is a hydrogen atom or a group selected from unsubstituted or substituted alkyl, for example methyl, trifluoromethyl, 3-methylsulfonamidopropyl, methyl- or phenyl-sulfonylmethyl, carboxytetrafluoroethyl; unsubstituted or substituted aryl, for example phenyl, 3,5-di-chlorophenyl, o-methanesulfonamidophenyl, 4-methanesulfonylphenyl, 2(2'-hydroxyethyl)phenyl, 2-hydroxy-4-methylphenyl, 2-hydroxymethylphenyl, o-hydroxybenzyl; a carbonyl-containing group, for example an alkylamino-, alkoxy-, aryloxy- or hydroxyalkylamino-carbonyl; or contains an imidazolyl, pyrazolyl, triazolyl, tetrazolyl, pyridyl, pyridinium, piperidinyl, morpholino, quinolinium or a quinolinyl group or R₁ may include a group which splits off a photographically useful fragment, such as a phenylmercaptotetrazole or a 5-or 6-nitroindazole group. Examples of some of these are disclosed in US 5,328,801.

More preferably R₁ contains a morpholino group and especially has the formula -CONH(CH₂)ₙ-morpholino, wherein n is 0-4 and is conveniently 3.

R₂ and R₃ are preferably hydrogen atoms or alkyl groups with p being preferably 1 and R₄, R₅ and R₆ are preferably hydrogen, alkyl, alkoxy, alkylthio, trifluoromethyl or methylsulfonamido groups, with q being preferably 0 or 1 and m being preferably 0. R₇ is preferably hydrogen or an alkyl group, optionally substituted with, for example, a dialkylamino group.

When X is S=0 or C-NH it is preferred that n is 1 and that (link₁) comprises an arylamino group or an arylaminocarbonyl group, preferably a phenylaminocarbonyl group, which may be substituted in the ring, for example, with one or more alkyl, carboxyl groups or halogen atoms. When X is C it is preferred that n is 0 such that no (link₁) group is present.

The (link₂) group preferably comprises a polyalkylene group comprising alkylene groups, preferably methylene groups, typically four or six, which may be separated by one or more O or S atoms. For example (link₂) may be (CH₂)₄, (CH₂)₆, (CH₂)₂S(CH₂)₂ or (CH₂)₂O(CH₂)₂O(CH₂)₂. Alternatively (link₂) may be a polyalkylene oxide chain extending from an even number of methylene groups such as (CH₂CH₂O)₁₄CH₂CH₂ or may comprise, for example, a CH₂C₆H₄CH₂ group.

The anionic counterion may be selected from any well known in the art and may typically be selected from Cl⁻, Br⁻, I⁻, CF₃COO⁻, CH₃SO₃⁻ and TsO⁻.

Unless otherwise specifically stated, substituent groups usable on molecules herein include any groups, whether substituted or unsubstituted, which do not destroy properties necessary for photographic utility.

When the term "group" is applied to the identification of a substituent containing a substitutable hydrogen, it is intended to encompass not only the substituent's unsubstituted form, but also its form further substituted with any group or groups as herein mentioned.

Suitably, the group may be halogen or may be bonded to the remainder of the molecule by an atom of carbon, silicon, oxygen, nitrogen, phosphorus, or sulfur. The substituent may be, for example, halogen, such as chlorine, bromine or fluorine; nitro; hydroxyl; cyano; carboxyl; or groups which may be further substituted, such as alkyl, including straight or branched chain alkyl, such as methyl, trifluoromethyl, ethyl, *t*-butyl, 3-(2,4-di-t-pentylphenoxy) propyl, and tetradecyl; alkenyl, such as ethylene, 2-butene; alkoxy, such as methoxy, ethoxy, propoxy, butoxy, 2-methoxyethoxy, *sec*-butoxy, hexyloxy, 2-ethylhexyloxy, tetradecyloxy, 2-(2,4-di-*t*-pentylphenoxy)ethoxy, and 2-dodecyloxyethoxy; aryl such as phenyl, 4-t-butylphenyl, 2,4,6-trimethylphenyl, naphthyl; aryloxy, such as phenoxy, 2-methylphenoxy, alpha- or beta-naphthyloxy, and 4-tolyloxy; carbonamido, such as acetamido, benzamido, butyramido, tetradecanamido, alpha-(2,4-di-*t*-pentylphenoxy)acetamido, alpha-(2,4-di-*t*-pentylphenoxy)butyramido, alpha-(3-pentadecylphenoxy)hexanamido, alpha-(4-hydroxy-3-*t*-butylphenoxytetradecanamido, 2-oxo-pyrrolidin-1-yl, 2-oxo-5-tetradecylpyrrolidin-1-yl, N-methyltetradecanamido, N-succinimido, N-phthalimido, 2,5-dioxo-1-oxazolidinyl, 3-dodecyl-2,5-dioxo-1-imidazolyl, and N-acetyl-N-dodecylamino, ethoxycarbonylamino, phenoxycarbonylamino, benzyloxycarbonylamino, hexadecyloxycarbonylamino, 2,4-di-t-butylphenoxycarbonylamino, phenylcarbonylamino, 2,5-(di-*t*-pentylphenyl)-carbonylamino, *p*-dodecylphenylcarbonylamino, *p*-toluylcarbonylamino, N-methylureido, N,N-dimethylureido, N-methyl-N-dodecylureido, N-hexadecylureido, N,N-dioctadecylureido, N,N-di-octyl-N'-ethylureido, N-phenylureido, N,N-diphenylureido, N-phenyl-N-*p*-toluyl-ureido, N-(m-hexadecylphenyl)ureido, N,N-(2,5-di-*t*-pentylphenyl)-N'-ethylureido, and *t*-butylcarbonamido; sulfonamido, such as methylsulfonamido, benzenesulfonamido, *p*-toluylsulfonamido, *p*-dodecylbenzenesulfonamido, N-methyltetradecylsulfonamido, N,N-di-propylsulfamoylamino, and hexadecylsulfonamido; sulfamoyl, such as N-methylsulfamoyl, N-ethylsulfamoyl, N,N-di-propylsulfamoyl, N-hexadecylsulfamoyl, N,N-dimethylsulfamoyl; N-[3-(do-decyloxy)propyl]-sulfamoyl, N-[4-(2,4-di*t*-pentylphenoxybutyl]sulfamoyl, N-methyl-N-tetradecylsulfamoyl, and N-dodecylsulfamoyl; carbamoyl, such as N-methylcarbamoyl, N,N-dibutylcarbamoyl, N-octadecylcarbamoyl, N-[4-(2,4-di-*t*-pentylphenoxy)butyl]carbamoyl, N-methyl-N-tetradecylcarbamoyl, and N,N-dioctylcarbamoyl; acyl, such as acetyl, (2,4-di-t-amylphenoxy)acetyl, phenoxycarbonyl, *p*-dodecyloxyphenoxycarbonyl, methoxycarbonyl, butoxycarbonyl, tetradecyloxycarbonyl, ethoxycarbonyl, benzyloxycarbonyl, 3-pentadecyloxycarbonyl, and dodecyloxycarbonyl; sulfonyl, such as methoxysulfonyl, octyloxysulfonyl, tetradecyloxysulfonyl, 2-ethylhexyloxysulfonyl, phenoxysulfonyl, 2,4-di-*t*-pentylphenoxysulfonyl, methylsulfonyl, octylsulfonyl, 2-ethylhexylsulfonyl, dodecylsulfonyl, hexadecylsulfonyl, phenylsulfonyl, 4-nonylphenylsulfonyl, and *p-*toluylsulfonyl; sulfonyloxy, such as dodecylsulfonyloxy, and hexadecylsulfonyloxy; sulfinyl, such as methylsulfinyl, octylsulfinyl, 2-ethylhexylsulfinyl, dodecylsulfinyl, hexadecylsulfinyl, phenylsulfinyl, 4-nonylphenylsulfinyl, and *p*-toluylsulfinyl; thio, such as ethylthio, octylthio, benzylthio, tetradecylthio, 2-(2,4-di-*t*-pentylphenoxy)ethylthio, phenylthio, 2-butoxy-5-t-octylphenylthio, and *p*-tolylthio; acyloxy, such as acetyloxy, benzoyl-oxy, octadecanoyloxy, *p*-dodecylamidobenzoyloxy, N-phenylcarbamoyloxy, N-ethylcarbamoyloxy, and cyclohexylcarbonyloxy; amine, such as phenylanilino, 2-chloroanilino, diethylamine, dodecylamine; imido, such as 1 (N-phenylimido) ethyl, N-succinimido or 3-benzylhydantoinyl; phosphate, such as dimethylphosphate and ethylbutylphosphate; phosphite, such as diethyl and dihexylphosphite; a heterocyclic group, a heterocyclic oxy group or a heterocyclic thio group, each of which may be substituted and which contain a 3 to 7-membered heterocyclic ring composed of carbon atoms and at least one hetero atom selected from the group consisting of oxygen, nitrogen and sulfur, such as 2-furyl, 2-thienyl, 2-benzimidazolyloxy or 2-benzothiazolyl; quaternary ammonium, such as triethylammonium; and silyloxy, such as trimethylsilyloxy.

If desired, the substituents may themselves be further substituted one or more times with the described substituent groups. The particular substituents used may be selected by those skilled in the art to attain the desired photographic properties for a specific application and can include, for example, hydrophobic groups, solubilizing groups, blocking groups, releasing or releasable groups and groups which adsorb to silver halide. Generally, the above groups and substituents thereof may include those having up to 48 carbon atoms, typically 1 to 36 carbon atoms and usually less than 24 carbon atoms, but greater numbers are possible depending on the particular substituents selected.

Generally the synthesis of a compound of formula (I) will produce an amount of a compound of formula (II) in a greater or lesser amount. For the purpose of achieving the advantages of this invention it has been found surprisingly that a number of relative amounts of these two components can be used with advantage, without isolation of either component, providing a significant benefit in the synthesis thereof. Although not critical to the function of the invention, for ease of synthesis it is convenient if the compound of formula (II) comprises two identical moieties linked by (link)₂.

In some embodiments, the nucleators of the invention may be selected from the following:-

### Compounds of formula (I)

### Compounds of formula (II)

The photographic material of the invention may also contain a booster compound to enhance the ultrahigh contrast and to promote activity, although as previously mentioned the use of the nucleators described herein means that the amount of any such booster can be substantially reduced. Alternatively the booster compound can be present in the developer solution.

One class of such boosters are amines which
(1) comprise at least one secondary or tertiary amino group, and
(2) have an n-octanol/water partition coefficient (log P) of at least one, preferably at least three, and most preferably at least four,
log P being defined by the formula: $log P = log \frac{\left[{X}_{octanol}\right]}{\left[{X}_{water}\right]}$ wherein X is the concentration of the amino compound.

Preferably such an amine contains within its structure a group comprising at least three repeating ethyleneoxy units as described in US Patent 4,975,354. These units are preferably directly attached to the nitrogen atom of a tertiary amino group.

Included within the scope of the amino compounds which may be utilised in this invention are monoamines, diamines and polyamines. The amines can be aliphatic amines or they can include aromatic or heterocyclic moieties. Aliphatic, aromatic and heterocyclic groups present in the amines can be substituted or unsubstituted groups. Preferably, the amine boosters are compounds having at least 20 carbon atoms.

Preferred amino compounds for inclusion in photographic materials of the invention are bis-tertiary amines which have a partition coefficient of at least three and a structure represented by the formula:-

R¹R²N -(CH₂CH₂O)ₙ -CH₂CH₂-NR³R⁴

wherein n is an integer from 3 to 50, and more preferably 10 to 50;
R¹, R², R³ and R⁴ are, independently, alkyl groups of 1 to 8 carbon atoms, or
R¹ and R² taken together represent the atoms necessary to complete a heterocyclic ring, and/or R³ and R⁴ taken together represent the atoms necessary to complete a heterocyclic ring.

A particularly preferred booster for use in photographic materials of the invention or in the developer therefor is the booster B 1 wherein in the above formula R¹, R², R³ and R⁴ are each n-propyl groups and n is 14, i.e. the structure:-

Another preferred group of amino compounds is that of bis-secondary amines which have a partition coefficient of at least three and a structure represented by the formula:-

RHN(CH₂CH₂O)ₙ-CH₂CH₂-NHR

wherein n is an integer from 3 to 50, and more preferably 10 to 50, and
each R is, independently, a linear or branched, substituted or unsubstituted, alkyl group of at least 4 carbon atoms.

Particular amines suitable as booster compounds are listed in EP-A-0 364 166.

Other types of boosters are described in US Patent No. 5,744,279 as having one of the formulae:-

(a) Y((X)ₙ-A-B)ₘ

wherein Y is a group which adsorbs to silver halide,
X is a divalent linking group composed of hydrogen, carbon, nitrogen and sulfur atoms,
A is a divalent linking group,
B is an amino group which may be substituted or an ammonium group of a nitrogen-containing heterocyclic group,
m is 1, 2 or 3 and
n is 0 or 1,

(b) R¹R²N-R3-(X)ₙ-SMₓ

wherein R¹ and R² are each hydrogen or an aliphatic group, or R¹ and R² may together form a ring,
R³ is a divalent aliphatic group,
X is a divalent heterocyclic ring having at least one nitrogen, oxygen or sulfur atom as heteroatom,
n is 0 or 1,
M is hydrogen or an alkali metal atom, alkaline earth metal atom, a quaternary ammonium, quaternary phosphonium atom or an amidino group, and
x is 1 when M is a divalent atom;
said compound optionally being in the form of an addition salt;
a phosphonium structure as disclosed in col. 8 of USP 5,744,279 and as exemplified by the following formula:- or a pyridinium structure as disclosed in col. 21 of the afore-mentioned US Patent as exemplified by the following formula:-

The nucleator(s) and optionally the booster compound can be incorporated in the photographic element, for example in a silver halide emulsion layer. Alternatively they can be present in a hydrophilic colloid layer of the photographic element, preferably a hydrophilic layer which is coated to be adjacent to the emulsion layer in which the effects of the nucleator are desired. They can however be present in the photographic element distributed between or among emulsion and hydrophilic colloid layers, such as undercoating layers, interlayers and overcoating layers.

Typically the nucleator(s) may be present in the photographic material in a total amount of from about 1µmol/m² to about 100µmol/m², preferably 3µmol/m² to 50µmol/m², more preferably 5µmol/m² to 20µmol/m². Corresponding amounts for the booster are from 0 mol/m² to about 1mmol/m², preferably 10µmol/m² to 100µmol/m², most preferably 30µmol/m² to 100µmol/m².

When a compound of formula (I) is in combination with a compound of formula (II), any relative proportions of the components may achieve the advantages of the invention. However preferably the amount of compound of formula (I): compound of formula (II) is in the range from about 10:90 to about 90:10, preferably from about 20:80 to about 80:20. Conveniently however for simplicity of synthesis the compound of formula (II) is produced in excess and generally the relative amounts of the components are then in the range about 15:85 to about 30:70.

The emulsions employed in photographic materials of the invention and the addenda added thereto, the binders, supports etc. may be as described in Research Disclosure Item 36544, September 1994, published by Kenneth Mason Publications, Emsworth, Hants, PO10 7DQ, United Kingdom, which will be identified hereinafter by the term "Research Disclosure."

The hydrophilic colloid may be gelatin or a gelatin derivative, polyvinylpyrrolidone or casein and may contain a polymer. Suitable hydrophilic colloids and vinyl polymers and copolymers are described in Section IX of the Research Disclosure. Gelatin is the preferred hydrophilic colloid.

The photographic materials may also contain an overcoat hydrophilic colloid layer which may also contain a vinyl polymer or copolymer located as the last layer of the coating (furthest from the support). It contains one or more surfactants to aid coatability and may also contain some form of matting agent. The vinyl polymer is preferably an acrylic polymer and preferably contains units derived from one or more alkyl or substituted alkyl acrylates or methacrylates, alkyl or substituted alkyl acrylamides, or acrylates or acrylamides containing a sulfonic acid group.

The photographic materials of the invention preferably contain an antihalation layer which may be on either side of the support, preferably on the opposite side of the support from the emulsion layer. In a preferred embodiment an antihalation dye is contained in the hydrophilic colloid underlayer. The dye may also be dissolved in or dispersed in the underlayer. Suitable dyes are listed in the Research Disclosure disclosed above.

The emulsions are preferably chemically sensitised, for example with both sulfur and gold. The latent-image forming grains can be bromoiodide, chlorobromoiodide, bromide, chlorobromide, chloroiodide or chloride, preferably chlorobromide. They should be preferably be spectrally sensitised. More than one type of spectrally sensitised silver halide grain may be present and hence grains sensitised to different spectral regions may be present in the emulsion layer.

The coating may be made by blending two or more emulsion melts containing grains of the required spectral sensitivity, allowing the production of multi-wavelength sensitive products and giving rise to manufacturing cost advantages through both material and inventory reduction. Combining the different emulsion grains within one layer can give improvements in process sensitivity over multilayer graphics nucleated systems, as described in EP-A-0 682 288.

The silver halide grains may be doped with rhodium, ruthenium, iridium or other Group VIII metals either alone or in combination, preferably at levels in the range 10⁻⁹ to 10⁻³, preferably 10⁻⁶ to 10⁻³ mole metal per mole of silver. The grains may be mono- or poly-disperse. The preferred Group VIII metals are rhodium and/or iridium and ammonium pentachlororhodate may conveniently be used.

The present photographic materials are particularly suitable for exposure by red or infra-red laser diodes, light emitting diodes or gas lasers, e.g. a helium/neon or argon laser.

The light-sensitive silver halide contained in the photographic elements can be processed following exposure to form a visible image by associating the silver halide with an aqueous alkaline medium in the presence of a developing agent contained in the medium or the element. The photographic elements of this invention can be processed in conventional developers as opposed to specialised developers sometimes employed in conjunction with lithographic photographic elements to obtain very high contrast images. When the photographic elements contain incorporated developing agents the elements can be processed in the presence of an activator, which can be identical to the developer in composition, but otherwise lacking a developing agent.

Very high contrast images can be obtained at pH values below 11, preferably in the range of from 10.0 to 10.8, preferably in the range of 10.3 to 10.5 and especially at pH 10.4.

The developers are typically aqueous solutions, although organic solvents, such as diethylene glycol, can also be included to facilitate the solution of organic components. The developers contain one or a combination of conventional developing agents, such as, for example, a polyhydroxybenzene, such as dihydroxybenzene; aminophenol, paraphenylenediamine; ascorbic acid, erythorbic acid and derivatives thereof; pyrazolidone, pyrazolone, pyrimidine, dithionite and hydroxylamine.

It is preferred to employ hydroquinone and 3-pyrazolidone developing agents in combination or an ascorbic acid-based system. An auxiliary developing agent exhibiting superadditive properties may also be used. The pH of the developers can be adjusted with alkali metal hydroxides and carbonates, borax and other basic salts. It is, as previously mentioned, a particular advantage of the present invention that the use of a nucleator as described herein reduces the sensitivity of the photographic material to changes in this developer pH.

To reduce gelatin swelling during development, compounds such as sodium sulfate can be incorporated into the developer. Chelating and sequestering agents, such as ethylenediaminetetraacetic acid or its sodium salt, can be present. Generally any conventional developer can be used in the practice of this invention. Specific illustrative photographic developers are disclosed in the Handbook of Chemistry and Physics, 36^{th} Edition, under the title "Photographic Formulae" at page 30001 *et seq*. and in "Processing Chemicals and Formulas." 6^{th} Edition, published by Eastman Kodak Company (1963).

The invention will now be described with reference to the following examples which are in no way to be considered as limiting the scope thereof.

### Example 1

The following preparation of nucleator (M1) is illustrative for the nucleators of this invention of formula (A). All the compounds prepared had infra-red, mass and NMR spectra which were in accordance with pure samples of the desired products.

### b2,6-Dimethyl-3-(4-[3-morpholinopropylcarbamoylcarbonylhydrazino]-phenylsulfamoyl)phenylcarbamoylmethyl 3-(6-Pyrid-3-ylamidohexamethylenecarbamoyl)pyridinium chloride hydrochloride. (M1).

### Step 1: Ethyl 4-nitrophenylhydrazinooxalate

4-Nitrophenylhydrazine (15.31g, 0.1mol) was dissolved in a mixture of dry tetrahydrofuran (THF) (100 ml) and dry dimethylformamide (25 ml). N,N-dimethylaniline (12.11 g, 0.1 mol) was added and the dark solution stirred. Ethyl oxalyl chloride (13.65 g, 0.1 mol) in THF (20ml) was added in a thin stream with stirring. The reaction evolved considerable heat and the temperature of the mixture was maintained at ambient by immersion in an ice/acetone bath. The mixture was stirred at room temperature for 2h. The volume of the solution was reduced on the rotary evaporator (to about 60 ml) and the mixture run slowly into a stirred mixture of ice/water (420 ml) and concentrated hydrochloric acid (1 ml). The tacky brown solid was filtered, washed with water, dried first at the pump and then in the vacuum oven overnight at 40C over potassium hydroxide. The product was obtained as a brown solid (23.64g; yield 93.3%).

### Step 2 : N-(3-Morpholinopropylcarbamoylcarbonyl)-4-nitrophenylhydrazine

Ethyl 4-nitrophenylhydrazinooxalate (58.9 g, 0.232 mol) was mixed with isopropanol (300 ml) and N-(3-aminopropyl)morpholine (33.54 g, 0.232 mol). The red mixture was heated at reflux for 2h, checked by MS to ascertain that all the starting material had been consumed and allowed to cool to room temperature. A dark red crystalline deposit was obtained and removed by filtration and air-dried. The product was obtained as a dark red solid (72.73 g; yield 89.2%).

### Step 3 : N-(3-morpholinopropylcarbamoylcarbonyl)-4-aminophenylhydrazine

A flask was charged with N-(3-morpholinopropylcarbamoylcarbonyl)-4-nitrophenylhydrazine (100g, 0.285mol) and palladium on charcoal (5g, 50% wet with water). THF (960ml) and dimethylacetamide (480ml) were added and the flask was placed on a CAMILE^{™} Automated Reactor. A program was run to heat to 55C over 30min. and a solution of ammonium formate (120g in 120ml water) was added over a period of 1h keeping the temperature at 55C plus or minus 5 degrees. After completion of the addition the mixture was stirred and heated at 55C for 2h, filtered warm (45-50C) through Kieselguhr and the catalyst residue washed with THF. The THF was concentrated off on the rotary evaporator and a heavy, yellow precipitate resulted, which was filtered and washed with isopropanol. The residue was dried (vac/50C) to give a pale yellow solid (54g; yield 60%)

### Step 4 : 3-Chloroacetamido-2,4-dimethyl-N-(4-[3-morpholinopropylcarbamoylcarbonylhydrazino]phenyl)benzenesulfonamide hydrochloride

N-(3-morpholinopropylcarbamoylcarbonyl) 4-aminophenylhydrazine (34.02g, 0.105 mol) was dissolved in a mixture of THF and dimethylacetamide (120ml/400ml) under nitrogen with stirring. 3-Choroacetamido-2,4-dimethylbenzenesulfonyl chloride (31.13 g, 0.105 mol) was added portionwise as a solid while the reaction mixture was stirred and cooled in an ice/acetone bath. The mixture was stirred for several hours. An MS was run which indicated that the required product had been formed. The solution was rotary evaporated to remove the THF. The resulting dimethylacetamide solution was poured into stirred isopropanol (1.51). The resulting pink solid was filtered off and dried under vacuum to give a brownish glass (60.03g, yield 92.6%).

### Step 5: 1,6-Dipyrid-3-ylamidohexane

Nicotinic acid (80g, 0.65mol) was dissolved in THF (780 ml) and triethylamine (65.63g, 0.65 mol) was added. The solution was cooled in an ice-bath (0-5C) and ethyl chloroformate (70.53g, 0.65 mol) was added dropwise, with stirring, over 30 min., keeping the temp below 5C. The mixture was stirred for a further 60 min. at ice-bath temperature and then a solution of 1,6-hexanediamine (37.76g, 0.325mol) in acetonitrile (780ml) was added in one portion. The reaction mixture was stirred at ambient temperature over night then checked by MS to ascertain that the reaction was complete. The white precipitate was removed by filtration and washed well with water to remove triethylamine hydrochloride and any residual traces of nicotinic acid and then dried in vacuum oven at 40C. The product was obtained as a white solid (45.31g; yield 42.7%).

### Step 6: 2,6-Dimethyl-3-(4-[3-morpholinopropylcarbamoylcarbonylhydrazino]-phenylsulfamoyl)phenylcarbamoylmethyl 3-(6-Pyrid-3-ylamidohexamethylenecarbamoyl)pyridinium chloride hydrochloride. (M1).

A 250ml flask was charged with 3-chloroacetamido-2,4-dimethyl-N-(4-[3-morpholinopropylcarbamoylcarbonylhydrazino]phenyl)benzene-sulfonamide hydrochloride (16g, 0.0275mol) dissolved in 100 ml dimethyl-acetamide. 1,6-Dipyrid-3-ylamidohexane (9g, 0.0275 mol) was added and the solution was degassed with nitrogen for 15min. before being heated to 70C and then held at 70C with stirring under nitrogen for 24 h. The hot reaction mixture was poured into stirred acetonitrile (11). A pinkish precipitate resulted. The mixture was stirred for 1 h before filtering and air drying the product at ambient temperature over night and then under vacuum at 40C. The product was obtained as a brown glass (22.2g; yield 90%).

The product comprised M1 and N1 in the ratio of 86:14 i.e. it comprised primarily the compound of formula (I).

Different relative proportions of the components can be achieved by varying the amounts of the reactants in step 6. For example doubling the amount of the morpholino compound in that step compared with the dipyridino compound and increasing the reaction temperature results in ratios of (M1): (N1) in the range 80:20 to 90:10, i.e. the compound of formula (II) is then in excess.

### Example 2

### Preparation of Nucleating Agent (M13) and (N8)

Analogously with the above preparation, the following synthetic route for the preparation of the nucleator (M13), is illustrative for the nucleators for this invention of formula (B):-

This synthesis also produces the dimeric molecule (N8).

### Example 3

### Preparation of Nucleating Agent (M15)

Analogously, the following synthetic route for the preparation of nucleator (M15, is illustrative for the nucleators of this invention of formula (C): No compound of formula (II) is prepared in this synthesis.

### Example 4

### Preparation of Coatings

The film coatings prepared consisted of a polyethylene terephthalate (ESTAR^{™}) support on which was coated an emulsion layer and a protective gel overcoat.

The emulsion layer consisted of 3.3g Ag/m² of a 70:30 chlorobromide cubic monodispersed emulsion (0.18µm edge length) uniformly doped with ammonium pentachlororhodate at 0.17mg/Agmol and chemically sensitized with sulfur and gold, and also included 60mg/m² of booster B1.

The emulsion was spectrally sensitized with 350mg/Agmol of 1H-benzimidazole-1-propanesulfonic acid, 2-((1,3-diethyl-tetrahydro-4,6-dioxo-2-thioxo-5(2H)-pyrimidinylidene) ethylidene)-3-ethyl-2,3-dihydro-, sodium salt. Other addenda included were 270mg/Agmol of 2-mercapto-methyl-5-carboxy-4-hydroxy-6-methyl-1,3,3a,7-tetra-azaindene and 23mg/Agmol 1-(3-acetamidophenyl)-5-mercaptotetrazole. The layer also contained 2.00g/m² gel, and 0.6g/m² of copolymer methacrylate: 2-acrylamido-2-methylpropanesulfonic acid: sodium salt of 2-acetoxyethyl-methacrylate (88:5:7 by weight).

Three further coatings were made to the same formulation except that in each instance a solution of nucleating agent was added to the emulsion before coating at a rate sufficient to provide a total nucleating agent concentration of 0.327g nucleating agent/mol Ag, as follows:-
solution A 0.6% of a comparison hydrazide nucleating agent C1, currently used in commercial product, in 30% aqueous methanol;
solution B 0.6% of 82% M1 and 18% N1 in water
solution C 0.6% of 8% M1 and 92% N1 in water.
C1 has the formula:- wherein X = S-(CH₂CH₂O)₄-C₈H₁₇

### Example 5

### Evaluation of Coatings

### (i) Sensitometric data

The coatings were evaluated by exposing through a 0.1 increment step wedge with a 10⁻⁶ sec. flash sensitometer fitted with a P11 filter (which simulates an argon-ion laser exposing source) and then processed in Kodak RA2000^{™} Developer (diluted 1+2) with development times of 20s. and 40s. at 35C. Comparisons of the sensitometry for the coatings described above were made as shown in Table I.

**TABLE I**

| **Sensitometric and Process latitude data** | | | | | |
|---|---|---|---|---|---|
| **Nucl.** | **Dev.time** | **D**_{**min**} | **D**_{**max**} | **Sp2.0** | **Gr2.0** |
| **None** | 20s | 0.017 | 6.60 | 1.09 | 15.12 |
| | 40s | 0.024 | 6.85 | 1.21 | 14.63 |
| **A** | 20s | 0.017 | 6.85 | 1.28 | 18.48 |
| | 40s | 0.024 | 6.85 | 1.55 | 32.78 |
| **B** | 20s | 0.018 | 6.85 | 1.19 | 18.89 |
| | 40s | 0.021 | 6.85 | 1.27 | 19.53 |
| **C** | 20s | 0.016 | 6.85 | 1.22 | 26.72 |
| | 40s | 0.020 | 6.85 | 1.30 | 29.75 |

### In Table I (and Table II) the following abbreviations are used:-

**D**_{**min**}- minimum density:
**D**_{**max**}- maximum density
**Sp0.6 -** toe speed, measured as the relative logE exposure required to produce a density of 0.6 above Dₘᵢₙ
**Sp2.0** - measured as the relative logE exposure required to produce a density of 2.0 above Dₘᵢₙ
**PrD -** practical density, measured as the density achieved at an exposure 0.4 logE units higher than the Sp0.6 value
**Gr2.0 -** measured as the gradient between density points 1.5 and 2.5 above Dₘᵢₙ
**USC** - upper scale contrast, measured as the gradient between density points 2.5 and 4.0 above Dₘᵢₙ
**EC** - effective contrast, measured as the gradient between density points 0.1 and 2.5 above Dₘᵢₙ.
**Spread -** chemical spread, measured as the rate of increase in line width (µ/s) produced when development time is increased from 20s at 35C.

### (ii) Sensitometric evaluation

It will be seen from Table I that the measured low-density contrast (Gr2.00) for all the nucleated coatings was significantly higher at the same development time than that for the coating with no nucleator present, demonstrating effective nucleation by all the coatings.

However, increasing the development time for the coating containing the comparison nucleator C1 (solution A) caused a large increase in contrast, showing that the system was not robust to changes in processing conditions. With both the solutions B and C, containing nucleating agents according to the invention, the increase in contrast with development time was very much reduced. This reduction in process variability provided by the inventive nucleators is a highly desirable improvement. While solution C (in which N1 predominates) was somewhat more active than solution B (predominantly M1), adequate nucleation, matching that of the comparison nucleator C1, was still observed with solution B.

The increased stability towards process changes was also demonstrated by the measured speed parameters Sp2.0, where again it can be seen that the increased speed observed at the longer process time was smaller for the two coatings using nucleating agents according to the invention than it was for comparison nucleator C1.

### Example 6

### Preparation of Coatings

The film coatings prepared consisted of a polyethylene terephthalate (ESTAR^{™}) support (with an antihalation pelloid layer on its rear surface) on which was coated an emulsion layer, a gel interlayer, and a protective overcoat.

The emulsion layer consisted of 2.8g Ag/m² of a 70:30 chlorobromide cubic monodispersed emulsion (0.16µm edge length) uniformly doped with ammonium pentachlororhodate at 4.4x10⁻⁷ moles per Ag mole and dipotassium hexachloroiridate at 6x10⁻⁷ moles per Ag mole and chemically sensitized with sulfur and gold. The emulsion was spectrally sensitized with 350mg/Agmol of sensitizing dye S1. Other addenda included were 243mg/Agmol of 2-mercapto-methyl-5-carboxy-4-hydroxy-6-methyl-1,3,3a,7-tetra-azaindene and 23mg/Agmol 1-(3-acetamidophenyl)-5-mercaptotetrazole. The layer also contained 1.4gm² gel, and 0.4g/m² of copolymer methacrylate: 2-acrylamido-2-methylpropanesulfonic acid: sodium salt of 2-acetoxyethylmethacrylate (88:5:7 by weight).

### Senstitizing dye S1, wherein R₄ is methyl and R₅ is isopropyl

An interlayer illustrative of the present invention consisted of 0.65g/m² gel, 0.2g/m² copolymer methacrylate: 2-acrylamido-2-methylpropane sulfonic acid: sodium salt of 2-acetoxyethyl methacrylate (88:5:7 by weight), 96mg/m² 3,5-disulphocatechol, 44mg/m² hydroquinone, 7.5mg/m² of nucleating agent and 60mg/m² booster compound B1.

The overcoat contained 1 g/m² gel with matte beads and surfactants to aid coatability.

Various coatings were made by changing the interlayer formulation as indicated in Table II below. Different nucleating agents were used with variations in the percentage of components of formulae (I) and (II).

### Example 7

### Evaluation of Coatings

### (i) Sensitometric data

The coatings were evaluated by exposing through a 0.1 increment step wedge with a 10⁻⁶s. flash sensitometer fitted with a W29 filter (which simulates an red exposing source) and then processed in Kodak^{™} RA2000 Developer (diluted 1+2) for 20s. at 35C. Comparisons of the sensitometry for the coatings described above were made as shown in Table II

**TABLE II**

| **Sensitometric data** | | | | | | | | | |
|---|---|---|---|---|---|---|---|---|---|
| **Nucl.** | **Level mg/m**^{**2**} | **II:I ratio** | **D**_{**min**} | **PrD** | **Sp0.6** | **EC** | **USC** | **C.Spr.** | **20-30sDeltaSp** |
| A | 7.5 | 60:40 | 0.016 | 5.61 | 1.14 | 12.55 | 27.94 | 0.41 | 0.10 |
| B | 7.5 | 64:36 | 0.014 | 5.71 | 1.13 | 14.43 | 33.12 | 0.39 | 0.07 |
| C | 7.5 | 75:25 | 0.013 | 5.75 | 1.15 | 12.04 | 35.13 | 0.42 | 0.08 |
| D | 7.5 | 84:16 | 0.014 | 5.64 | 1.14 | 13.02 | 31.74 | 0.41 | 0.07 |
| E | 7.5 | 87:13 | 0.015 | 5.77 | 1.13 | 13.38 | 37.23 | 0.33 | 0.07 |
| F | 7.5 | 91:9 | 0.015 | 5.70 | 1.13 | 15.17 | 34.38 | 0.36 | 0.07 |
| A | 10 | 60:40 | 0.015 | 5.85 | 1.17 | 14.87 | 31.99 | 0.50 | 0.09 |
| B | 10 | 64:36 | 0.016 | 5.72 | 1.15 | 14.83 | 27.63 | 0.46 | 0.09 |
| C | 10 | 75:25 | 0.015 | 5.74 | 1.17 | 14.99 | 31.71 | 0.46 | 0.08 |
| D | 10 | 84:16 | 0.013 | 5.88 | 1.17 | 14.25 | 31.21 | 0.46 | 0.08 |
| E | 10 | 87:13 | 0.014 | 5.84 | 1.15 | 14.67 | 31.34 | 0.50 | 0.08 |
| F | 10 | 91:9 | 0.015 | 5.86 | 1.16 | 13.83 | 32.53 | 0.45 | 0.08 |

### (ii) Sensitometric evaluation

From the data presented it was clear that there were only small differences (generally within experimental error) between the samples containing the variations in compounds of formulae (I) and (II).

All the samples coated showed values for the effective contrast (EC) over 10 showing good nucleation, producing high contrast and good dot quality. The upper scale contrast (USC) indicated a very high shoulder contrast with all samples. The Dₘᵢₙ values were all minimal and the practical density figures above 5 showing good density achieved and the chemical spread was within acceptable limits.

### (iii) Process latitude evaluation

The coatings tabulated above were also evaluated for process latitude to development time. The results are also shown in Table II wherein it was seen that there is negligible variation in speed between a development time of 20s. and 30s.

## Claims

1. An ultrahigh contrast photographic material comprising a support bearing a silver halide emulsion layer, containing a hydrazide nucleating agent in the emulsion layer or a hydrophilic colloid layer, **characterised in that** the nucleating agent of formula (I) has one of the formulae:- or
wherein Z¹ and Z² are the same or different and each is a nicotinamide residue, at least one of which is positively charged;
Y is a substituted aryl or heterocyclic ring;
one of A₁ and A₂ is a hydrogen atom and the other is a hydrogen atom, an acyl group or an alkyl- or aryl-sulfonyl group, any of which groups may be substituted;
BG is a blocking group;
L is a linking group;
T is an anionic counterion
and n is 1 or 2.

2. A photographic material according to claim 1 **characterised in that** the nucleating agent has one of the formulae:- wherein
R₁CO comprises a blocking group and R₁ is selected from a hydrogen atom, and an unsubstituted or substituted alkyl, aryl, alkoxy, aryloxy, alkoxy- or aryloxy-carbonyl and alkyl- or aryl-aminocarbonyl group; or R₁ is or contains an unsubstituted or substituted heterocyclic group, having a 5- or 6-membered ring containing at least one nitrogen, oxygen or sulfur atom, wherein the ring may be linked either directly to the carbonyl group or via an alkyl, alkoxy, carbonyl, amino- or alkylamino-carbonyl group and wherein the ring may be fused to an unsubstituted or substituted benzene ring;
R₂ and R₃ are independently selected from hydrogen and an unsubstituted or substituted alkyl or aryl group and p is 0 or 1;
R₄ and R₅ and each R₆, which may be the same or different, are independently selected from hydrogen, halogen, hydroxy, cyano and an unsubstituted or substituted alkyl, aryl, heterocyclyl, alkoxy, acyloxy, aryloxy, carbonamido, sulfonamido, ureido, thioureido, semicarbazido, thiosemicarbazido, urethane, quaternary ammonium, alkyl- or aryl-thio, alkyl- or aryl-sulfonyl, alkyl- or arylsulfinyl, carboxyl, alkoxy- or aryloxy-carbonyl, carbamoyl, sulfamoyl, phosphonamido, diacylamino, imido or acylurea group, a group containing a selenium or a tellurium atom and a group having a tertiary sulfonium structure;
each m is the same or different and is an integer from 0 to 4;
q is an integer from 0 to 4;
each R₇ is the same or different and is independently selected from hydrogen and an unsubstituted or substituted alkyl or aryl group
X is selected from C, S=O and C-NH;
(link₁) is selected from an unsubstituted or substituted alkylene, polyalkylene, aryl, arylaminocarbonyl or heterocyclyl group and n is 0 or 1; and
(link₂) is a linking group selected from an unsubstituted or substituted polyalkylene, polyalkylene oxide, polyalkylene containing one or more heteroatoms selected from nitrogen, oxygen and sulfur, separated from each other by alkylene groups, or an unsubstituted or substituted polyalkylene in which the alkylene groups are separated by an unsubstituted or substituted aryl or heterocyclic ring and
T⁻ is an anionic counterion.

3. A photographic material according to claim 2 **characterised in that**
R₁ is a hydrogen atom or a methyl, trifluoromethyl, 3-methylsulfonamidopropyl, methyl- or phenyl-sulfonylmethyl, carboxytetrafluoroethyl, phenyl, 3,5-di-chlorophenyl, o-methanesulfonamidophenyl, 4-methanesulfonylphenyl, 2(2'-hydroxyethyl)phenyl, 2-hydroxy-4-methylphenyl, 2-hydroxymethylphenyl, o-hydroxybenzyl, alkylamino-, alkoxy-, aryloxy- or hydroxyalkylamino-carbonyl; or contains an imidazolyl, pyrazolyl, triazolyl, tetrazolyl, pyridyl, pyridinium, piperidinyl, morpholino, quinolinium or a quinolinyl, phenylmercaptotetrazole or a 5-or 6-nitroindazole group.

4. A photographic material according to claim 3 **characterised in that** R₁ is the group -CONH(CH₂)ₙ-morpholino, wherein n is 0 to 4.

5. A photographic material according to any one of claims 2 to 4 **characterised in that** R₂ and R₃ are independently selected from hydrogen atoms or alkyl groups.

6. A photographic material according to any one of claims 2 to 5 **characterised in that** R₄, R₅ and R₆ are independently selected from hydrogen, alkyl, alkoxy, alkylthio, trifluoromethyl or methylsulfonamido groups.

7. A photographic material according to any one of claims 2 to 6 **characterised in that** R₇ is hydrogen, an alkyl group or an alkyl group substituted with a dialkylamino group.

8. A photographic material according to any one of claims 2 to 7 **characterised in that** X is S=0 or C-NH and n is 1.

9. A photographic material according to any one of claims 2 to 7 **characterised in that** X is C and n is 0.

10. A photographic material according to any one of claims 2 to 8 **characterised in that** (link₁) comprises an unsubstituted or substituted arylamino group or an arylaminocarbonyl group.

11. A photographic material according to any one of claims 2 to 10 **characterised in that** (link₂) comprises a (CH₂)₄, (CH₂)₆, (CH₂)₂S(CH₂)₂, (CH₂)₂O(CH₂)₂O(CH₂)₂, (CH₂CH₂O)₁₄CH₂CH₂ or CH₂C₆H₄CH₂ group.

12. A photographic material according to any one of claims 8, 10 and 11 **characterised in that** the nucleating agent has the formula:-

13. A photographic material according to any one of the preceding claims **characterised in that** the nucleating agent of formula (I) is in combination with a nucleating agent of formula (II), which comprises a dimeric molecule comprising two monomers linked by a linking group, each monomer of which (a) may be the same or different and (b) comprises a hydrazide moiety and a nicotinamide moiety.

14. A photographic material according to claim 13 **characterised in that** the nucleating agent of formula (II) has one of the formulae:- or
wherein each monomer linked by linking group L is the same or different;
Z is a positively charged nicotinamide residue; and Y, A₁, A₂, BG, L and T are as defined in claim 1.

15. A photographic material according to claim 14 **characterised in that** the nucleating agent of formula (II) has one of the formulae:-
wherein each R₁, R₂, R₃, R₄, R₅, R₆, R₇, m, n, p, q, X and (link₁) is the same or different and, together with (link₂) and T, is as defined in any one of claims 2 to 11.

16. A photographic material according to claim 15 **characterised in that** the nucleating agent of formula (II) has the formula:-

17. A photographic material according to any one of claims 1-8 and 10 to 16 **characterised in that** the nucleating agent comprises a combination of the compounds as defined in claims 12 and 16.

18. A photographic material according to any one of the preceding claims **characterised in that** it also contains, in the emulsion layer or a hydrophilic colloid layer, a booster compound.

19. A photographic material according to claim 18 **characterised in that** the booster compound is an amine booster.

20. A photographic material according to claim 19 **characterised in that** the booster compound is

21. A photographic material according to any one of the preceding claims **characterised in that** the nucleator(s) is present in the photographic material in a total amount of from about 1 µmol/m² to about 100µmol/m²

22. A photographic material according to any one of claims 13 to 21 **characterised in that** the relative proportion of compound of formula (I) to formula (II) is from about 10:90 to about 90:10.

23. A photographic material according to claim 22 wherein the amount of compound of formula (II) is greater than the amount of formula (I) and the relative proportion of compound of formula (I) to formula (II) is from about 15:85 to about 30:70.

24. A process of forming a photographic image having ultrahigh contrast which comprises imagewise exposing a photographic material comprising a support bearing a silver halide emulsion layer and processing it with an alkaline developer **characterised in that** it is developed in the presence of a nucleating agent as defined in any one of claims 1 to 12 or a combination of nucleating agents as defined in any one of claims 13 to 17.

25. A process according to claim 24 **characterised in that** the photographic material is developed in the presence of a booster compound.

## Patentansprüche

1. Fotografisches Material von ultrahohem Kontrast mit einem Träger, auf dem sich eine Silberhalogenidemulsionsschicht befindet, das in der Emulsionsschicht oder in einer hydrophilen Kolloidschicht ein Hydrazid-Keimbildungsmittel enthält, **dadurch gekennzeichnet, dass** das Keimbildungsmittel der Formel (I) eine der Formeln aufweist: oder
worin Z¹ und Z² gleich oder verschieden sind und jeweils stehen für einen Nicotinamidrest, von denen mindestens einer positiv geladen ist;
Y ein substituierter Aryl- oder heterozyklischer Ring ist;
einer der Reste A₁ und A₂ ein Wasserstoffatom ist und der andere ein Wasserstoffatom, eine Acylgruppe oder eine Alkyl- oder Arylsulfonylgruppe, wobei jede Gruppe substituiert sein kann;
BG eine blockierende Gruppe ist;
L eine verbindende Gruppe ist;
T ein anionisches Gegenion darstellt
und n gleich 1 oder 2 ist.

2. Fotografisches Material nach Anspruch 1, **dadurch gekennzeichnet, dass** das Keimbildungsmittel eine der Formeln aufweist: worin
R₁CO eine blockierende Gruppe ist und R₁ ausgewählt ist aus einem Wasserstoffatom und einer unsubstituierten oder substituierten Alkyl-, Aryl-, Alkoxy-, Aryloxy-, Alkoxy- oder Aryloxycarbonyl- und Alkyl- oder Arylaminocarbonylgruppe; oder R₁ steht für eine oder enthält eine unsubstituierte oder substituierte, heterozyklische Gruppe mit einem 5- oder 6-gliedrigen Ring mit mindestens einem Stickstoff-, Sauerstoff- oder Schwefelatom, wobei der Ring entweder direkt an die Carbonylgruppe gebunden ist oder über eine Alkyl-, Alkoxy-, Carbonyl-, Amino- oder Alkylaminocarbonylgruppe und worin der Ring an einen unsubstituierten oder substituierten Benzolring ankondensiert sein kann;
R₂ und R₃ unabhängig voneinander ausgewählt sind aus einem Wasserstoffatom und einer unsubstituierten oder substituierten Alkyl- oder Arylgruppe und p für 0 oder 1 steht;
R₄ und R₅ und jede Gruppe R₆, die gleich oder verschieden sein können, unabhängig voneinander ausgewählt sind aus einem Wasserstoff- oder Halogenatom oder einer Hydroxy-, Cyano- und einer unsubstituierten oder substituierten Alkyl-, Aryl-, Heterocyclyl-, Alkoxy-, Acyloxy-, Aryloxy-, Carbonamido-, Sulfonamido-, Ureido-, Thioureido-, Semicarbazido-, Thiosemicarbazido-, Urethan-, quaternären Ammonium-, Alkyl- oder Arylthio-, Alkyl- oder Arylsulfonyl-, Alkyl- oder Arylsulfinyl-, Carboxyl-, Alkoxy- oder Aryloxycarbonyl-, Carbamoyl-, Sulfamoyl-, Phosphonamido-, Diacylamino-, Imido- oder Acylharnstoffgruppe, einer Gruppe mit einem Selen- oder einem Telluratom und einer Gruppe mit einer tertiären Sulfoniumstruktur;
m jeweils die gleiche oder eine verschiedene Bedeutung hat und für eine ganze Zahl von 0 bis 4 steht;
q eine ganze Zahl von 0 bis 4 ist;
die Reste R₇ gleich oder verschieden sind und unabhängig voneinander ausgewählt sind aus Wasserstoff sowie einer unsubstituierten oder substituierten Alkyl- oder Arylgruppe;
X ausgewählt ist aus C, S=O und C-NH;
(link₁) ausgewählt ist aus einer unsubstituierten oder substituierten Alkylen-, Polyalkylen-, Aryl-, Arylaminocarbonyl- oder Heterocyclylgruppe und n steht für 0 oder 1; und worin
(link₂) eine verbindende Gruppe ist, die ausgewählt ist aus einem unsubstituierten oder substituierten Polyalkylen, Polyalkylenoxid, Polyalkylen mit einem oder mehreren Heteroatomen, ausgewählt aus Stickstoff, Sauerstoff und Schwefel und getrennt voneinander durch Alkylengruppen oder einem unsubstituierten oder substituierten Polyalkylen, in dem die Alkylengruppen voneinander getrennt sind durch einen unsubstituierten oder substituierten Aryl- oder heterozyklischen Ring und worin
T⁻ ein anionisches Gegenion ist.

3. Fotografisches Material nach Anspruch 2, **dadurch gekennzeichnet, dass** R₁ steht für ein Wasserstoffatom oder eine Methyl-, Trifluoromethyl-, 3-Methylsulfonamidopropyl-, Methyl- oder Phenylsulfonylmethyl-, Carboxytetrafluoroethyl-, Phenyl-, 3,5-Dichlorophenyl-, o-Methansulfonamidophenyl-, 4-Methansulfonylphenyl-, 2(2'-Hydroxyethyl) phenyl-, 2-Hydroxy-4-methylphenyl-, 2-Hydroxymethylphenyl-, o-Hydroxybenzyl-, Alkylamino-, Alkoxy-, Aryloxy- oder Hydroxyalkylaminocarbonylgruppe; oder eine Imidazolyl-, Pyrazolyl-, Triazolyl-, Tetrazolyl-, Pyridyl-, Pyridinium-, Piperidinyl-, Morpholino-, Chinolinium- oder eine Chinolinyl-, Phenylmercaptotetrazol- oder eine 5-oder 6-Nitroindazolgruppe enthält.

4. Fotografisches Material nach Anspruch 3, **dadurch gekennzeichnet, dass** R₁ die Gruppe -CONH(CH₂)ₙ-Morpholino ist, worin n für 0 bis 4 steht.

5. Fotografisches Material nach einem der Ansprüche 2 bis 4, **dadurch gekennzeichnet, dass** R₂ und R₃ unabhängig voneinander ausgewählt sind aus Wasserstoffatomen oder Alkylgruppen.

6. Fotografisches Material nach einem der Ansprüche 2 bis 5, **dadurch gekennzeichnet, dass** R₄, R₅ und R₆ unabhängig voneinander ausgewählt sind aus Wasserstoff, Alkyl-, Alkoxy-, Alkylthio, Trifluoromethyl- oder Methylsulfonamidogruppen.

7. Fotografisches Material nach einem der Ansprüche 2 bis 6, **dadurch gekennzeichnet, dass** R₇ steht für Wasserstoff, eine Alkylgruppe oder eine Alkylgruppe, die durch eine Dialkylaminogruppe substituiert ist.

8. Fotografisches Material nach einem der Ansprüche 2 bis 7, **dadurch gekennzeichnet, dass** X steht für S=0 oder C-NH und dass n steht für 1.

9. Fotografisches Material nach einem der Ansprüche 2 bis 7, **dadurch gekennzeichnet, dass** X steht für C und n steht für 0.

10. Fotografisches Material nach einem der Ansprüche 2 bis 7, **dadurch gekennzeichnet, dass** (link₁) eine unsubstituierte oder substituierte Arylaminogruppe oder eine Arylaminocarbonylgruppe umfasst.

11. Fotographisches Material nach einem der Ansprüche 2-10 **dadurch gekennzeichnet, dass** (link₂) umfasst eine (CH₂)₄, (CH₂)₆, (CH₂)₂S(CH₂)₂, (CH₂)₂O(CH₂)₂O(CH₂)₂, (CH₂CH₂O)₁₄CH₂CH₂ oder CH₂C₆H₄CH₂ Gruppe.

12. Fotografisches Material nach einem der Ansprüche 8, 10 und 11, **dadurch gekennzeichnet, dass** das Keimbildungsmittel die Formel aufweist:

13. Fotografisches Material nach einem der vorstehenden Ansprüche, **dadurch gekennzeichnet, dass** das Keimbildungsmittel der Formel (I) in Kombination mit einem Keimbildungsmittel der Formel (II) vorliegt, das ein dimeres Molekül umfasst mit zwei Monomeren, die miteinander verbunden sind durch eine verbindende Gruppe, wobei jedes Monomer (a) gleich oder verschieden sein kann und (b) einen Hydrazidrest und einen Nicotinamidrest aufweist.

14. Fotografisches Material nach Anspruch 13, **dadurch gekennzeichnet, dass** das Keimbildungsmittel der Formel (II) eine der Formeln aufweist: oder
worin jedes Monomer, das angebunden ist durch die verbindende Gruppe L, gleich oder verschieden ist;
Z ein positiv geladener Nicotinamidrest ist; und
Y, A₁, A₂, BG, L und T die in Anspruch 1 angegebene Bedeutung haben.

15. Fotografisches Material nach Anspruch 14, **dadurch gekennzeichnet, dass** das Keimbildungsmittel der Formel (II) einer der Formeln entspricht:
worin R₁, R₂, R₃, R₄, R₅, R₆, R₇, m, n, p, q, X und (link₁) gleich oder verschieden sind und gemeinsam mit (link₂) und T die in einem der Ansprüche 2 bis 11 angegebene Bedeutung haben.

16. Fotografisches Material nach Anspruch 15, **dadurch gekennzeichnet, dass** das Keimbildungsmittel der Formel (II) der Formel entspricht:

17. Fotografisches Material nach einem der Ansprüche 1 - 8 und 10 bis 16, **dadurch gekennzeichnet, dass** das Keimbildungsmittel eine Kombination von den Verbindungen, wie in Ansprüchen 12 und 16 angegeben, enthält.

18. Fotografisches Material nach einem der vorstehenden Ansprüche, **dadurch gekennzeichnet, dass** es ferner in der Emulsionsschicht oder in einer hydrophilen Kolloidschicht eine Booster-Verbindung enthält.

19. Fotografisches Material nach Anspruch 18, **dadurch gekennzeichnet, dass** die Booster-Verbindung ein Amin-Booster ist.

20. Fotografisches Material nach Anspruch 19, **dadurch gekennzeichnet, dass** die Booster-Verbindung eine Verbindung der Formel ist:

21. Fotografisches Material nach einem der vorstehenden Ansprüche, **dadurch gekennzeichnet, dass** das oder die Keimbildungsmittel in dem fotografischen Material in einer Gesamtmenge von etwa 1 µMol/m² bis etwa 100 µMol/m² vorliegen.

22. Fotografisches Material nach einem der Ansprüche 13 bis 21, **dadurch gekennzeichnet, dass** das relative Verhältnis von Verbindung der Formel (I) zur Verbindung der Formel (II) bei etwa 10:90 bis etwa 90:10 liegt.

23. Fotografisches Material nach Anspruch 22, in dem die Menge der Verbindung der Formel (II) größer ist als die Menge der Verbindung der Formel (I) und in dem das relative Verhältnis der Verbindung der Formel (I) zur Verbindung der Formel (II) bei etwa 15:85 bis etwa 30:70 liegt.

24. Verfahren zur Herstellung eines fotografischen Bildes mit ultrahohem Kontrast, das umfasst die bildweise Exponierung eines fotografischen Materials mit einem Träger, auf dem sich eine Silberhalogenidemulsionsschicht befindet und die Entwicklung des Materials mit einem alkalischen Entwickler, **dadurch gekennzeichnet, dass** das Material entwickelt wird in Gegenwart eines Keimbildungsmittels, wie in einem der Ansprüche 1 bis 12 definiert, oder in Gegenwart einer Kombination von Keimbildungsmitteln, wie in einem der Ansprüche 13 bis 17 definiert.

25. Verfahren nach Anspruch 24, **dadurch gekennzeichnet, dass** das fotografische Material in Gegenwart einer Booster-Verbindung entwickelt wird.

## Revendications

1. Matériau photographique à contraste ultra élevé comprenant un support portant une couche d'émulsion aux halogénures d'argent, contenant un agent de nucléation hydrazide dans la couche d'émulsion ou une couche de colloïde hydrophile, **caractérisé en ce que** l'agent de nucléation de formule (I) est représenté par l'une des formules :
où Z¹ et Z² sont identiques ou différents et chacun est un résidu nicotinamide, dont au moins un est de charge positive ;
Y est un groupe aryle ou un hétérocycle substitué ;
et l'un des groupes A₁ et A₂ est un atome d'hydrogène et l'autre est un atome d'hydrogène, un groupe acyle ou un groupe alkyl- ou aryl-sulfonyle, l'un quelconque de ces groupes pouvant être substitué ;
BG est un groupe bloquant ;
L est un groupe de liaison ;
T est un contre-ion anionique
et n est 1 ou 2.

2. Matériau photographique selon la revendication 1, **caractérisé en ce que** l'agent de nucléation est représenté par l'une des formules :
où R₁CO comprend un groupe bloquant et R₁ est choisi parmi un atome d'hydrogène, et un groupe alkyle, aryle, alcoxy, aryloxy, alcoxy- ou aryloxy-carbonyle et un groupe alkyl- ou aryl-aminocarbonyle substitué ou non ; ou R₁ est ou contient un groupe hétérocyclique substitué ou non ayant un cycle à 5 ou 6 membres contenant au moins un atome d'azote, d'oxygène ou de soufre, où le cycle peut être relié soit directement au groupe carbonyle soit par l'intermédiaire d'un groupe alkyle, alcoxy, carbonyle, amino- ou alkylamino-carbonyle et où le cycle peut être condensé sur un cycle benzène substitué ou non ;
R₂ et R₃ sont indépendamment choisis parmi l'hydrogène et un groupe alkyle ou aryle substitué ou non et p est 0 ou 1 ;
R₄ et R₅ et chacun des groupes R₆, qui peuvent être identiques ou différents, sont indépendamment choisis parmi l'hydrogène, l'halogène, un radical hydroxy, cyano et un groupe alkyle, aryle, hétérocyclyle, alcoxy, acyloxy, aryloxy, carbonamido, sulfonamido, uréido, thiouréido, semicarbazido, thiosemicarbazido, uréthane, ammonium quaternaire, alkyl- ou aryl-thio, alkyl- ou aryl-sulfonyle, alkyl- ou aryl-sulfinyle, carboxyle, alcoxy- ou aryloxy-carbonyle, carbamoyle, sulfamoyle, phosphonamido, diacylamino, imido ou acylurée substitué ou non, un groupe contenant un atome de sélénium ou de tellure et un groupe ayant une structure sulfonium tertiaire ;
chaque groupe m est identique ou différent et est un entier de 0 à 4 ;
q est un entier de 0 à 4 ;
chaque groupe R₇ est identique ou différent et est indépendamment choisi parmi l'hydrogène et un groupe alkyle ou aryle substitué ou non ;
X est choisi parmi C, S=O et C-NH ;
(link₁) est choisi parmi un groupe alkylène, polyalkylène, aryle, arylaminocarbonyle ou hétérocyclyle substitué ou non et n est 0 ou 1 ; et
(link₂) est un groupe de liaison choisi parmi un groupe polyalkylène, polyoxyalkylène substitué ou non, polyalkylène contenant un ou plusieurs hétéroatomes choisis parmi l'azote, l'oxygène et le soufre, séparés les uns des autres par des groupes alkylène ou un groupe polyalkylène substitué ou non, dans lequel les groupes alkylène sont séparés par un groupe aryle ou un hétérocycle substitué ou non, et
T⁻ est un contre-ion anionique.

3. Matériau photographique selon la revendication 2, **caractérisé en ce que**
R₁ est un atome d'hydrogène ou un groupe méthyle, trifluorométhyle, 3-méthylsulfonamidopropyle, méthyl- ou phényl-sulfonylméthyle, carboxytétrafluoroéthyle, phényle, 3,5-di-chlorophényle, o-méthanesulfonamidophényle, 4-méthanesulfonylphényle, 2(2'-hydroxyéthyl)phényle, 2-hydroxy-4-méthylphényle, 2-hydroxyméthylphényle, o-hydroxybenzyle, alkylamino-, alcoxy-, aryloxy- ou hydroxyalkylaminocarbonyle ; ou contient un groupe imidazolyle, pyrazolyle, triazolyle, tétrazolyle, pyridyle, pyridinium, pipéridinyle, morpholino, quinolinium, ou un groupe quinolinyle, phényl-mercaptotétrazole ou un groupe 5- ou 6-nitroindazole.

4. Matériau photographique selon la revendication 3, **caractérisé en ce que** R₁ est le groupe -CONH(CH₂)ₙ-morpholino, où n est de 0 à 4.

5. Matériau photographique selon l'une quelconque des revendications 2 à 4, **caractérisé en ce que** les groupes R₂ et R₃ sont indépendamment choisis parmi les atomes d'hydrogène ou les groupes alkyle.

6. Matériau photographique selon l'une quelconque des revendications 2 à 5, **caractérisé en ce que** R₄, R₅ et R₆ sont indépendamment choisis parmi l'hydrogène, les groupes alkyle, alcoxy, alkylthio, trifluorométhyle ou méthylsulfonamido.

7. Matériau photographique selon l'une quelconque des revendications 2 à 6, **caractérisé en ce que** R₇ est l'hydrogène, un groupe alkyle ou un groupe alkyle substitué par un groupe dialkylamino.

8. Matériau photographique selon l'une quelconque des revendications 2 à 7, **caractérisé en ce que** X est S=0 ou C-NH et n est 1.

9. Matériau photographique selon l'une quelconque des revendications 2 à 7, **caractérisé en ce que** X est C et n est 0.

10. Matériau photographique selon l'une quelconque des revendications 2 à 8, **caractérisé en ce que** (link₁) comprend un groupe arylamino ou arylaminocarbonyle substitué ou non.

11. Matériau photographique selon l'une quelconque des revendications 2 à 10, **caractérisé en ce que** (link₂) comprend un groupe (CH₂)₄, (CH₂)₆, (CH₂)₂S(CH₂)₂, (CH₂)₂O(CH₂)₂O(CH₂)₂, (CH₂CH₂O)₁₄CH₂CH₂ ou CH₂C₆H₄CH₂.

12. Matériau photographique selon l'une quelconque des revendications 8, 10 et 11, **caractérisé en ce que** l'agent de nucléation est représenté par la formule :

13. Matériau photographique selon l'une quelconque des revendications précédentes, **caractérisé en ce que** l'agent de nucléation de formule (I) est combiné à un agent de nucléation de formule (II), qui comprend une molécule dimère comprenant deux monomères reliés par un groupe de liaison, dont chaque monomère (a) peut être identique ou différent et (b) comprend un radical hydrazide et un radical nicotinamide.

14. Matériau photographique selon la revendication 13, **caractérisé en ce que** l'agent de nucléation de formule (II) est représenté par l'une des formules :
où chaque monomère relié par le groupe de liaison L est identique ou différent ;
Z est un résidu nicotinamide de charge positive ; et
Y, A₁, A₂, BG, L et T sont tels que définis dans la revendication 1.

15. Matériau photographique selon la revendication 14, **caractérisé en ce que** l'agent de nucléation de formule (II) est représenté par l'une des formules :
où chaque groupe R₁, R₂, R₃, R₄, R₅, R₆, R₇, m, n, p, q, X et (link₁) est identique ou différent, et ensemble avec (link₂) et T, sont tels que définis dans l'une quelconque des revendications 2 à 11.

16. Matériau photographique selon la revendication 15, **caractérisé en ce que** l'agent de nucléation de formule (II) est représenté par la formule :

17. Matériau photographique selon l'une quelconque des revendications 1 à 8, et 10 à 16, **caractérisé en ce que** l'agent de nucléation comprend une combinaison de composés telle que définie dans les revendications 12 et 16.

18. Matériau photographique selon l'une quelconque des revendications précédentes, **caractérisé en ce qu'**il contient également, dans la couche d'émulsion ou dans une couche de colloïde hydrophile, un composé amplificateur.

19. Matériau photographique selon la revendication 18, **caractérisé en ce que** le composé amplificateur est un amplificateur amine.

20. Matériau photographique selon la revendication 19, **caractérisé en ce que** le composé amplificateur est

21. Matériau photographique selon l'une quelconque des revendications précédentes, **caractérisé en ce que** le(s) nucléateur(s) est(sont) présent(s) dans le matériau photographique en une quantité totale comprise entre 1 µmole/m² environ et 100 µmoles/m² environ.

22. Matériau photographique selon l'une quelconque des revendications 13 à 21, **caractérisé en ce que** la proportion relative de composé de la formule (I) à la formule (II) est comprise entre 10:90 environ et 90:10 environ.

23. Matériau photographique selon la revendication 22, dans lequel la quantité de composé de formule (II) est supérieure à la quantité de composé de formule (I) et la proportion relative de composé de la formule (I) à la formule (II) est comprise entre 15:85 environ et 30:70 environ.

24. Procédé de formation d'une image photographique ayant un contraste ultra élevé qui consiste à exposer, conformément à l'image, un matériau photographique comprenant un support portant une couche d'émulsion aux halogénures d'argent et à le traiter avec un révélateur alcalin, **caractérisé en ce qu'**il est développé en présence d'un agent de nucléation tel que défini dans l'une quelconque des revendications 1 à 12 ou d'une combinaison d'agents de nucléation telle que définie dans l'une quelconque des revendications 13 à 17.

25. Procédé selon la revendication 24, **caractérisé en ce que** le matériau photographique est développé en présence d'un composé amplificateur.
